

## UNITED STATES PATENT OFFICE

2,174,573

PRODUCTION OF CRIMPED CELLULOSE  
DERIVATIVE YARNS

Donald Finlayson, Spondon, near Derby, England, assignor to Celanese Corporation of America, a corporation of Delaware

No Drawing. Application April 7, 1937, Serial No. 135,490. In Great Britain May 1, 1936

9 Claims. (Cl. 57—157)

This invention relates to improvements in filaments, yarns, fibres and the like and is more particularly concerned with the production of yarns exhibiting characteristics commonly associated 5 with natural fibres and especially wool.

In prior U. S. Patents Nos. 2,089,198 and 2,089,-199 and British Patent No. 464,981 I have described processes for imparting crimp to yarn by setting twist in the yarn while it is travelling, and 10 subsequently removing twist from the yarn. The twist to be inserted in the yarn may be a false twist, and the twist may be set in the yarn either while it is travelling in the course of the operation in which the twist is imparted or in the course of 15 the operation in which the twist is removed. The specifications all describe the application of the process to the treatment of yarns consisting of continuous filaments or yarns consisting of staple fibre which in the case of artificial material may 20 either be produced by cutting up continuous filaments and subsequently spinning the cut fibre into a yarn or may be produced by direct conversion from a continuous filament yarn, for example by the processes of U. S. Patents Nos. 2,077,078 and 2,077,079. Further, it is stated in the said specifications that the filaments (including fibres) contained in the basic yarn may be of a lustrous character or may be delustrated as by subjecting cellulose acetate or other cellulose derivative materials to hot aqueous liquors or liquors containing 25 thiocyanates or solvents for the cellulose derivative, so as to resemble more closely the finer qualities of natural staple fibres. By subjecting such 30 a yarn to the crimping process of the prior U. S. Patents Nos. 2,089,198 and 2,089,199 and British Patent No. 464,981 a product is produced which 35 has a subdued lustre, is crimped to some extent by the delustring treatment, and is further crimped by the twisting, setting and untwisting process. 40 Before or after the twisting, setting and untwisting, the yarn may, according to the processes of the prior specifications, be converted into a staple fibre yarn, as already indicated.

I have now found that a superior product, particularly as regards the crimp, may be obtained by 45 twisting cellulose derivative yarns, setting the twist, untwisting, and subsequently treating with hot aqueous media and particularly hot aqueous liquors. It appears that by applying the treatment with a hot aqueous medium after the twisting, setting and untwisting operation, a higher 50 degree of crimp is imparted than is the case when the treatment with the hot aqueous medium is applied before the twisting, setting and untwisting operation.

The yarn to be treated in accordance with the combined process of the present invention may be a continuous filament yarn or it may be a staple fibre yarn formed by any suitable process, for example by cutting continuous filaments to staple 5 lengths and subsequently spinning into a yarn, or it may be a yarn produced by direct conversion of a continuous filament yarn into a yarn containing staple fibre, as by the processes of U. S. Patents Nos. 2,077,078 and 2,077,079. Alternatively a continuous filament yarn may be twisted, set and untwisted and, either before or after the subsequent treatment with hot aqueous liquors, converted into a staple fibre yarn, as for example by the processes previously mentioned. When at an intermediate stage in the conversion to a staple fibre yarn the material exists in the form of staple fibres, the treatment with a hot aqueous medium 10 may be applied to the materials in this form and before spinning into a yarn.

The material constituting the yarn may be cellulose acetate or any other organic derivative of cellulose, for example cellulose formate, propionate or butyrate, or other organic esters or mixed esters of cellulose, or ethyl or benzyl cellulose or other cellulose ethers or mixed ethers of cellulose, or mixed ether-esters of cellulose. Where the material is at some stage converted into a staple fibre yarn, it may be mixed with fibres of materials other than cellulose derivatives, for example 15 regenerated cellulose, natural silk, wool, cotton or the like, the other fibre being either lustrous or non-lustrous as desired.

As a result of the treatment according to the present invention, the cellulose derivative materials have a subdued lustre. If the lustre is required to be reduced still more, the process may be combined with a special delustring treatment, for example by incorporating white pigments into the materials either during the spinning process for 20 producing the original filaments, i. e. by incorporating the pigment in the spinning solution, or as an aftertreatment applied to the materials, such aftertreatment being applied at any convenient stage.

While the present invention contemplates the treatment by the combined process of twisting, setting and untwisting, and subsequent treatment in hot aqueous liquor of cellulose derivative 25 yarns of any character, especially valuable results may be obtained by treating yarns containing filaments or fibres of flat cross-section. The filaments or fibres constituting the yarn may be wholly flat in cross-section or may contain a substantial proportion of flats (as opposed to the 30

bulbous type of cross-section), for example more than 50% and preferably more than 70 or 80% of flats. It is found that the hot aqueous treatment imparts a better crimp to such materials than materials consisting wholly of filaments or fibres having a bulbous cross-section. The filaments or fibres of flat cross-section may be produced by any convenient method. One method is to spin a cellulose derivative solution containing the cellulose derivative in a concentration lower than the minimum required to produce bulbous cross-section. In particular, in the case of a solution of cellulose acetate in acetone, a concentration of 24% or lower, down to say 20%, and especially a concentration about 22-23½% produces a good variety of filament for the purpose of the present invention.

The operation of twisting the yarns, setting the twist and untwisting may be effected according to any of the processes described in prior U. S. Patents Nos. 2,089,198 and 2,089,199 and British Patent No. 464,981, referred to above.

While the treatment with a hot aqueous medium may simply consist of a treatment in wet steam, it is preferred to employ a boiling or almost boiling aqueous liquor. Such a liquor may contain a wetting agent, as for example a water-soluble soap or a sulphonated oil, for instance Monopol soap or Turkey red oil, or other sulphonated higher aliphatic compound, for instance a sulphonated higher fatty acid or a sulphonated higher fatty alcohol, or true sulphonic acids of the higher members of the aliphatic series. The treatment may, for example, be a treatment at the boil for ½ hour to 1½ hours in water containing a small proportion, for example up to 1 gram per litre, of wetting agent. Preferably, after such treatment the material is given a final wash-off, for instance in ordinary water which may be warm or hot. Such a washing-off may be repeated several times.

The treatment with a hot aqueous liquor may be operated so as to exercise a control over the lustre of the final product. A treatment of a cellulose acetate material with a boiling solution as described above produces a substantial reduction in lustre. A similar treatment with boiling water produces a much smaller reduction in lustre but still results in a product of substantially reduced lustre. If desired, salts or sugars may be added to the aqueous liquor, for example in a concentration up to 10 or 20% so as to reduce the loss in lustre occasioned by the hot aqueous treatment. Thus, for example, I may dissolve up to 10% of sodium chloride or up to 20% of sodium sulphate in the liquor and obtain a product which has a very good lustre and, at the same time, is well crinkled or crimped. For further information relating to these salts or sugars which have the effect of protecting the lustre of the material, reference is made to U. S. Patents Nos. 1,765,581 and 1,808,061. If desired the treatment with a hot aqueous medium may take place under pressure so as to enable temperatures higher than 100° C. to be used.

It is preferable in order to obtain a yarn of very woolly characteristics to finish with a doubled yarn having a light doubling twist which is reverse in direction to any twist in the constituent yarns. The twist, if any, in the constituent yarns should also be light. It is further very advantageous to have the product in this form before applying the treatment with the hot aqueous medium. This form of product may result directly from a twisting, setting and untwisting

step. For example, two or three yarns having either no twist or each having a light degree of twist in the same direction may be twisted together with a relatively high degree of twist, the twist set, as for example by means of steam, and the doubled yarn then untwisted so as to leave in the final yarn a light doubling twist, reverse in direction to any original twist in the constituent yarns. Where, as is preferred, the twisting, setting and untwisting operation comprises the insertion of false twist, the production of a doubled yarn of the character referred to will take place in a separate operation, and may either precede or follow the twisting, setting and untwisting operation.

Generally, by a light twist is meant a twist of not more than 5 turns per inch. A doubled yarn of the character referred to may be built up, for example, by taking a number of single yarns, each having say 0 or up to 1 or 2 turns per inch, and doubling them together with a doubling twist of 2 turns per inch in the reverse direction to any initial twist in the singles. Again, where a product of very heavy denier is required, two doubling operations may be employed. Thus, a number of single yarns each having 1 turn per inch or less may be doubled together with a doubling twist of 1 turn per inch in the same direction, and a number of yarns so doubled together with a doubling twist of 2 turns per inch reverse in direction.

Similarly, where the process includes the step of converting the product to a yarn containing staple fibre, a doubled yarn having the above characteristics may be obtained directly during such conversion step. For example, a number of continuous filament yarns having no twist or a light twist in one direction may be converted into yarns containing staple fibre by the process of U. S. Patent No. 2,077,079, and a number of such yarns travelling from this direct conversion process doubled together with a light twist, reverse in direction to any original twist in the yarn.

Having described my invention what I desire to secure by Letters Patent is:

1. Process for the production of improved crimped yarns, which comprises subjecting yarns which have a basis of organic derivatives of cellulose to the operations of twisting, setting the twist and untwisting, and thereafter subjecting the material of the yarns to treatment in a bath of hot aqueous liquid whereby a higher degree of crimp is imparted thereto.

2. Process for the production of improved crimped yarns, which comprises converting continuous filament yarns which have a basis of organic derivatives of cellulose into staple fibre yarns, subjecting the staple fibre yarns to the operations of twisting, setting the twist and untwisting, and thereafter subjecting the staple fibre yarns to treatment in a bath of hot aqueous liquid whereby a higher degree of crimp is imparted thereto.

3. Process for the production of improved crimped yarns, which comprises subjecting yarns which have a basis of organic derivatives of cellulose to the operations of twisting, setting the twist and untwisting, and thereafter converting such yarns into staple fibre yarns and subjecting the staple fibre yarns to treatment in a bath of hot aqueous liquid whereby a higher degree of crimp is imparted thereto.

4. Process for the production of improved crimped yarns, which comprises converting continuous filament yarns which have a basis of or-

- ganic derivatives of cellulose into staple fibre 5  
yarns by cutting the filaments of such yarns  
without destroying the continuity of the yarns as  
a whole, subjecting the staple fibre yarns so pro-  
duced to the operations of twisting, setting the  
twist and untwisting, and thereafter subjecting  
the staple fibre yarns to treatment in a bath of  
hot aqueous liquid whereby a higher degree of  
crimp is imparted thereto.
- 10 5. Process for the production of improved  
crimped yarns, which comprises subjecting yarns  
which have a basis of organic derivatives of cel-  
lulose to the operations of twisting, setting the  
twist and untwisting, cutting the yarns into sta-  
15 ple fibres, and thereafter subjecting the staple  
fibres to treatment in a bath of hot aqueous liquid  
whereby a higher degree of crimp is imparted  
thereto and converting such staple fibres into  
yarn.
- 20 6. Process for the production of improved  
crimped yarns, which comprises subjecting a plu-  
rality of yarns which have a basis of organic de-  
rivatives of cellulose and at most a low twist to  
the operations of doubling, setting the doubling  
25 twist and untwisting to an extent which leaves a  
small doubling twist in the yarns reverse in di-  
rection to the initial twist in the yarns, and  
thereafter subjecting the products to treatment  
in a bath of hot aqueous liquid whereby a higher  
degree of crimp is imparted thereto.
7. Process for the production of improved  
crimped yarns, which comprises subjecting yarns  
which have a basis of organic derivatives of cel-  
lulose to the operations of twisting, setting the  
twist and untwisting, and thereafter subjecting 5  
the material of the yarns to treatment in a bath  
of aqueous liquid maintained at a temperature of  
the order of the boiling temperature of the liquid  
whereby a higher degree of crimp is imparted  
thereto.
8. Process for the production of improved  
crimped yarns, which comprises subjecting yarns  
which have a basis of organic derivatives of cel-  
lulose to the operations of twisting, setting the  
twist and untwisting, and thereafter subjecting 10  
the material of the yarns to treatment in a bath  
of hot aqueous liquid containing a salt whereby a  
higher degree of crimp is imparted thereto.
9. Process for the production of improved  
crimped yarns, which comprises subjecting yarns 15  
which have a basis of organic derivatives of cel-  
lulose to the operations of twisting, setting the  
twist and untwisting, and thereafter subjecting  
the material of the yarns to treatment in a bath  
of hot aqueous liquid containing a sugar where- 20  
by a higher degree of crimp is imparted thereto.

DONALD FINLAYSON.